

Dec. 19, 1933.

J. EMIG

1,939,961

METHOD OF MAKING LINOLEUM

Filed Jan. 26, 1932

3 Sheets-Sheet 1



John Emig,  
by his atty.,  
Bynes, Stetson, Pamplin & Bleeker

Dec. 19, 1933.

J. EMIG

1,939,961

METHOD OF MAKING LINOLEUM

Filed Jan. 26, 1932

3 Sheets-Sheet 2

*Fig. 4.*



*Fig. 3.*



INVENTOR

John Emig  
by his atty.  
Byers, Stetson, Paquette & Blodsch

Dec. 19, 1933.

J. EMIG

1,939,961

METHOD OF MAKING LINOLEUM

Filed Jan. 26, 1932

3 Sheets-Sheet 3

*Fig. 5.*



*Fig. 6.*



INVENTOR

John Emig,  
by his attorney,  
Byrnes, Stellino, Pannier & Blenko

## UNITED STATES PATENT OFFICE

1,939,961

## METHOD OF MAKING LINOLEUM

John Emig, Lancaster, Pa., assignor to Armstrong Cork Company, Lancaster, Pa., a corporation of Pennsylvania

Application January 26, 1932. Serial No. 588,872

22 Claims. (Cl. 154—25)

This invention relates to a method of making linoleum, the word "linoleum" being used as a word of general definition and not of limitation, and being intended to include other or equivalent materials.

In the production of linoleum having a marbled pattern great difficulty has heretofore been encountered in obtaining patterns having the desired appearance. The marbling processes heretofore employed have not given the characteristic veining which is desired. Furthermore, it has been extremely difficult to obtain continuously, or to reproduce at will, the general appearance, color and value of a given pattern. Frequently over a run of only a few days the general appearance of the marble pattern will have varied quite materially and this is commercially undesirable. A suitable marbling process should constantly produce material which, while it has the free veining and freedom from harsh mechanical effect that are necessary in a marble pattern, should nevertheless continue to produce marbles of the same general appearance and color value so that a piece made at one time from given materials can be used successfully with a piece made at another time from like materials.

I provide a process wherein an assemblage of strips of linoleum mix, constituting a pack, is subjected to pressure on the longitudinal edges of the strips, preferably by rolling. Where rolls are employed the direction of rolling is longitudinally of the strips. The effect of applying pressure to the edges of the strips in the pack is to buckle such strips and form the pack into an irregularly veined body. This pressure also consolidates the several buckled strips. After this first operation the bodies thus formed are cross rolled. The cross rolling further reduces the thickness of the body and effects a sidewise distortion and spreading of the exposed portions of the strips. A highly desirable marbling is thus obtained. It is desirable to maintain a differential between the temperature of the rolls in this operation, and also to operate them at slightly different peripheral speeds, as this has bearing on the amount of sidewise spreading at the surface and contributes to the final appearance.

The general tone of the pattern is determined by the make-up of the pack from which the sheets are made. Various colors will be used and the sheets may be of different thicknesses. Once the make-up of a pack has been determined, comparable marbles can be produced at will simply

by reproducing the pack and subjecting it to the process.

I have found in practice that in order to get the proper color effects and a satisfactory product it is important that the several sheets making up the pack be homogeneous throughout. I prefer on this account to limit the thickness of any given sheet to not more than about 1/8th of an inch. It may be and frequently is necessary in obtaining certain of the effects contemplated by my invention to use strips thicker than this. Where I desire a thick strip of a given color in the pack I make it up from several plies, none of which is more than about 1/8th of an inch thick. This insures homogeneity throughout.

In order to get the proper balance of colors in the design, I find it necessary to limit the ratio between the amounts of the different colors present. The base color should not be unduly subordinated to the variegated colors, nor should the variegating colors stand out too prominently. Where the variegating colors are darker than the base color, there is danger of them obliterating the base color in part, and hence the percentage of variegating color present is relatively small. I prefer to employ not more than about 10 or 12% of variegating color, and preferably in the neighborhood of 8%. I have found, for example, in a pattern employing white as a base color and black and gray for variegating colors, that there should be about 91 1/2% of base color and 8 1/2% of variegating color. On the other hand, where the variegating color is lighter than the base, there is considerable danger of the base color obliterating the variegating color. I therefore prefer that where the base color is darker than the variegating color it shall not constitute more than 75 to 85 per cent of the total mix. For example, in a pattern having a black base color and white and gray as variegating colors, I found it necessary to employ 26 1/2% of variegating color in order to get the desired effect, thus leaving only 73 1/2% of base color.

It is also important that the sheets of variegating color be relatively thin if fine hard lined graining is to be produced. When the packs are first rolled there is some flattening, and on cross rolling the colors are drawn out to some considerable extent. If the variegating sheets are relatively thick there is considerable breaking through of the base color on cross rolling. This produces a clouded effect, and in order to obtain fine hard lined graining I have found that the thickness of the variegating color sheets should not be greater than about 1/20th of an inch.

Cloudiness involving variegating color may be obtained by thickening the sheets of variegating color, but if it is desired to obtain a cloudy background with sharp contrasting color, the variegating color should be supplied in the form of relatively thin sheets, as above, and other steps taken to obtain cloudiness in the background. I prefer to employ a striated base sheet. For example, I have obtained a cloudy gray and white background by using a granular mix consisting of 5 parts of white and 3 parts of gray and calendering the same to produce a short choppy jaspé graining. This material is used for background color in making up the packs.

15 In the accompanying drawings illustrating more or less diagrammatically a present preferred manner of carrying out the invention,

Figure 1 is a perspective view, partly broken away, showing a pack;

20 Figure 2 is a perspective illustrating the rolling of pieces cut from such pack;

Figure 3 is a view showing more or less diagrammatically the appearance of the material after it has been subjected to rolling as shown in

25 Figure 2;

Figure 4 is a perspective view illustrating the cross rolling;

Figure 5 is a view of a piece of linoleum made from material produced by my process; and

30 Figure 6 is a view showing a piece of striated base material.

Figure 1 illustrates a block made by piling together sheets of unmatured linoleum mix. In this particular case the block is made up of white bands 2, gray bands 3 and black bands 4. It will be noted that the white bands are made up of a plurality of plies 2a. For reasons above stated, the piles 2a should not be more than 1/8th of an inch thick, and the bands 3 and 4 should not be more than about 1/16th of an inch thick. In practice I have employed sheets of the following thicknesses:

|         | Inches |
|---------|--------|
| White   | .120   |
| 45 Gray | .035   |
| Black   | .025   |

These thicknesses can be increased somewhat, particularly if the product is to be used in large blocks, or if a darker base color is employed. For 56 a pack such as shown in Figure 1, wherein the base color is lighter than the variegating colors, the percentage of variegating color is kept relatively low; in this case 8.5 percent of the pack. A record is made of the order of piling and of the 55 color and thickness of the sheets so that the blocks with the colors in predetermined arrangement can be made up at will.

The difference in effect as between a light and a dark base color is well illustrated by considering 60 two mixes which may be employed together. It is common to make linoleum patterns consisting of light and dark squares, and linoleum made according to my process from the above described block may be used to form the light squares of a 65 marble pattern. A dark block for forming the dark squares of the pattern has been made from sheets of the following thicknesses:

|         | Inches |
|---------|--------|
| Black   | .125   |
| 70 Gray | .070   |
| White   | .075   |

The percentage of black in the block is 73.5% and the percentage of variegating color is 26.5%. The degree of sharpness or hardness in the light

and the dark patterns produced from the above blocks is about the same.

The unmatured sheets tend to adhere to one another to a degree, and the block can be readily handled as a unit. Packs are cut off or guillotined from the block along the chain lines a. The packs thus produced will be made up of relatively narrow strips or sheet-like pieces of linoleum mix. In the drawings the packs are indicated by the reference character 5.

I have found in practice that for the production of linoleum in commercial gauges the thickness of the packs should be limited. For the production of linoleum of a thickness of 0.95 inches I have successfully employed packs 5/8ths of an inch thick. Generally speaking, the pack thickness should be from one-half to three-quarters of an inch.

10 Figure 2 shows the manner of subjecting the packs 5 to the first pressing operation. The packs are laid side by side on a table 6 and fed between calender rolls 7 and 8. In operation the bottom roll 7 is kept at a temperature of approximately 65° F. and the top roll 8 at a temperature of 100° F. There is also a difference of one tooth between the number of teeth in the pinions 9 connecting the calendar rolls together. This causes a wiping action which spreads the color to some extent. The drawings are not intended to be to scale, the thickness of the linoleum being exaggerated for clarity of illustration.

105 Figure 3 shows the manner of subjecting the packs 5 to the first pressing operation. The packs are laid side by side on a table 6 and fed between calender rolls 7 and 8. In operation the bottom roll 7 is kept at a temperature of approximately 65° F. and the top roll 8 at a temperature of 100° F. There is also a difference of one tooth between the number of teeth in the pinions 9 connecting the calendar rolls together. This causes a wiping action which spreads the color to some extent. The drawings are not intended to be to scale, the thickness of the linoleum being exaggerated for clarity of illustration.

110 The rolling of the slabs 5 serves to buckle the individual strips making up the packs. The packs also adhere to one another so that there is produced a relatively wide sheet of veined linoleum composition. The veins run generally parallel and are reasonably straight, as shown in Figure 3, which it will be understood is diagrammatic only. The buckling of the strips is indicated at 10 in Figure 4. In the first rolling operation the packs are reduced to 1/4th to 1/6th of their original thickness. I have successfully used 5/8ths inch thick packs and reduced to 1/8th inch sheets.

115 The sheet of linoleum mix formed by the rolling operation of Figure 2 is cut into pieces of suitable length for cross rolling. The cross rolling machine is shown in Figure 4. It is a substantial duplicate of the machine of Figure 2 but it will be noted that the material is fed crosswise through the rolls so as to effect sidewise spreading of the veins.

120 In Figure 4 I have indicated the piling of the sheets one on top of the other. In practice I have employed 8 thicknesses, making a total thickness of 1 inch, and have cross rolled the same to the final thickness of .095. If desired, the sheets can be overlapped so as to make the operation of Figure 4 a continuous one.

125 It is in this operation that the preponderance of base color becomes most marked in the product. The percentage of white linoleum in the slab is apparent from Figure 1. The cross rolling so reduces the thickness of the material that the veins of gray and black are spread relatively far apart. They are also reshaped and take on the desired appearance. Some of the strips may be sharply divided from the adjacent color, while others blend softly into the adjacent color. There is no harshness to the pattern and no mechanical regularity.

130 Figure 5 shows squares 11 die cut from such material for the production of the white squares in a black and white marble pattern. The black squares 12 are made by using a pack in which

80

85

90

95

100

105

110

115

120

125

130

135

140

145

150

black predominates. In Figure 5 the squares have been assembled on a burlap backing 13 and consolidated and matured in the usual manner.

Figure 6 shows a piece of striated linoleum 5 which may be used instead of plain color, particularly where clouded effects in the background are desired.

My invention has been herein illustrated and described as applied to the production of a pattern simulating marble. It will be understood, however, that this is by way of illustration only as other desirable non-regular patterns may be produced by varying the make-up of the slabs which are employed. It will therefore be understood 10 that while I have illustrated and described a present preferred form of the invention it is not limited to such form but may be otherwise embodied or practiced within the scope of the following claims.

20 I claim:

1. In the method of making linoleum, the steps consisting in subjecting an assemblage of sheet-like strips of linoleum mix, which strips are of various colors and are arranged in a pack, to pressure in a direction generally in the plane of the strips and along their longitudinal edges, to thereby form the pack into a veined body.

2. In the method of making linoleum, the steps consisting in subjecting an assemblage of sheet-like strips of linoleum mix, which strips are of various colors and are arranged in a pack, to pressure in a direction generally in the plane of the strips and along their longitudinal edges, to thereby buckle the strips and form the pack into a veined body.

3. In the method of making linoleum, the steps consisting in subjecting an assemblage of sheet-like strips of linoleum mix, which strips are of various colors and are arranged in a pack, to pressure in a direction generally in the plane of the strips and along their longitudinal edges to thereby form the pack into a veined body, and then cross rolling such body.

4. In the method of making linoleum, the steps 45 consisting in forming a pack made up of sheet-like strips of linoleum mix on edge, which strips are of various colors, subjecting the pack to pressure, which pressure is applied in a direction generally in the plane of the strips and thereby forming the pack into an irregularly veined body.

5. In the method of making linoleum, the steps 55 consisting in subjecting an assemblage of sheet-like strips of linoleum mix, which strips are of various colors and are arranged in a pack, to pressure on the longitudinal edges of the strips and in a direction generally in the plane thereof, to thereby reduce the thickness of the pack and form it into an irregularly veined body.

6. In the method of making linoleum, the steps 60 consisting in assembling sheets of linoleum mix, which sheets are of different colors, into a block, cutting the same into packs made up of strips of various colors, and subjecting the packs to pressure on the longitudinal edges of such strips to thereby form the slab into a veined body.

7. In the method of making linoleum, the steps 70 consisting in assembling sheets of linoleum mix, which sheets are of different colors, into a block, cutting the same into packs made up of strips of various colors, and subjecting the packs to pressure on the longitudinal edges of such strips to thereby form the pack into a veined body, the packs being not thinner than about one-half inch.

8. In the method of making linoleum, the steps 75 consisting in assembling sheets of linoleum mix,

which sheets are of different colors, into a block, cutting the same into packs made up of strips of various colors, and subjecting the packs to pressure on the longitudinal edges of such strips to thereby form the pack into a veined body, the slabs being not thicker than about  $\frac{3}{4}$  of an inch.

9. In the method of making linoleum, the steps 80 consisting in forming linoleum mix into sheet-like pieces, forming at least one of such pieces from linoleum composition of different colors so as to obtain a multi-colored piece, forming the pieces into a pack wherein there are pieces of different color, and subjecting the pack to pressure on the longitudinal edges of the pieces to thereby form the pack into a veined body.

10. In the method of making linoleum, the steps 85 consisting in forming sheet-like strips of linoleum mix into a pack wherein there are bands of different color, at least some of the bands being made of a plurality of plies, and subjecting the pack to pressure on the longitudinal edges of the strips and in a direction generally in the plane thereof, to thereby form the pack into a veined body.

11. In the method of making linoleum, the steps 90 consisting in calendering linoleum mix into sheet-like pieces not more than about  $\frac{1}{8}$  inch in thickness, forming the pieces into a pack wherein there are bands of different color, and subjecting the pack to pressure on the longitudinal edges of the pieces and in a direction generally in the plane thereof, to thereby form the pack into a veined body.

12. In the method of making linoleum, the steps 95 consisting in calendering linoleum mix into sheet-like pieces not more than about  $\frac{1}{8}$  inch in thickness, forming the pieces into a pack wherein there are bands of different color, at least some of the bands being made of a plurality of plies, and subjecting the pack to pressure on the longitudinal edges of the pieces and in a direction generally in the plane thereof, to thereby form the pack into a veined body.

13. In the method of making linoleum, the steps 100 consisting in subjecting an assemblage of sheet-like strips of linoleum mix, which strips are of various colors and are arranged in a pack, to pressure on the longitudinal edges of the strips and in a direction generally in the plane thereof, to reduce the pack to  $\frac{1}{4}$ th- $\frac{1}{6}$ th of its original thickness, and thus forming a veined body.

14. In the method of making linoleum, the steps 105 consisting in forming linoleum mix into sheet-like pieces of different colors, at least one color constituting a base color and other colors constituting variegating colors, arranging the colors in a pack and subjecting the pack to pressure on the longitudinal edges of the pieces and in a direction generally in the plane thereof, to thereby form the pack into a veined body.

15. In the method of making linoleum, the steps 110 consisting in forming linoleum mix into sheet-like pieces of different colors, at least one color constituting the base color and other colors forming variegating colors, the base color being lighter than the variegating colors, forming the pieces into a pack wherein the variegating colors are not in excess of 12%, and subjecting the pack to pressure on the longitudinal edges of the pieces and in a direction generally in the plane thereof, to thereby form the pack into a veined body.

16. In the method of making linoleum, the steps 115 consisting in forming linoleum mix into sheet-like pieces of different colors, at least one

80

85

90

95

100

105

110

115

120

125

130

135

140

145

150

- color constituting a background color and other colors constituting variegating colors, the background color being darker than the variegating colors, forming the pieces into a pack wherein the background color does not exceed 85% of the whole, and subjecting the pack to pressure on the longitudinal edges of the pieces, and in a direction generally in the plane thereof, to thereby form the pack into a veined body.
17. In the method of making linoleum, the steps consisting in forming linoleum mix into sheet-like pieces of different colors, certain of the pieces constituting back-ground color and other pieces constituting variegating color, the pieces constituting variegating color being not more than about 1/16th inch in thickness, assembling the sheets into a pack, and subjecting the pack to pressure on the longitudinal edges of the pieces and in a direction generally in the plane thereof, to thereby form the pack into a veined body.
18. In the method of making linoleum, the steps consisting in assembling sheets of linoleum mix, which sheets are of different colors, into a block, cutting the same into packs made up of strips of various colors, subjecting the packs to pressure on the longitudinal edges of such strips to thereby form the slab into a veined body, and thereafter subjecting the body to cross rolling.
19. In the method of making linoleum, the steps consisting in subjecting an assemblage of sheet-like strips of linoleum mix, which strips are of various colors and are arranged in a pack, to rolling, the roll pressure being applied in such

manner as to deform the strips by compressing the edges of the strips toward one another, the direction of rolling being longitudinally of the strips.

20. In the method of making linoleum, the steps consisting in subjecting an assemblage of sheet-like strips of linoleum mix, which strips are of various colors and are arranged in a pack, to rolling, the roll pressure being applied in such manner as to deform the strips by compressing the edges of the strips toward one another, the direction of rolling being longitudinally of the strips, and thereafter subjecting the body to cross rolling.

21. In the method of making linoleum, the steps consisting in subjecting an assemblage of sheet-like strips of linoleum mix, which strips are of various colors and are arranged in a pack, to rolling, the roll pressure being applied in such manner as to deform the strips by compressing the edges of the strips toward one another, the direction of rolling being longitudinally of the strips, and maintaining the rolls at different temperatures.

22. In the method of making linoleum, the steps consisting in subjecting an assemblage of sheet-like strips of linoleum mix, which strips are of various colors and are arranged in a pack, to rolling, the roll pressure being applied in such manner as to deform the strips by compressing the edges of the strips toward one another, the direction of rolling being longitudinally of the strips, and operating the rolls a different speed.

JOHN EMIG. 116

- 40 115
- 45 120
- 50 125
- 55 130
- 60 135
- 65 140
- 70 145
- 75 150